

## 1

2,940,250

## HYPERGOLIC FUEL CONTAINING MERCAPTALS OR MERCAPTOLE

Manuel A. Pino, Richmond, and Paul C. Condit, Berkeley, Calif., assignors to California Research Corporation, San Francisco, Calif., a corporation of Delaware  
No Drawing. Filed Jan. 27, 1954, Ser. No. 406,617

2 Claims. (Cl. 60—35.4)

This invention relates to fuel compositions which are characterized by self-ignition when mixed with powerful oxidizing agents and to a method for initiating and maintaining combustion through the use of these fuels.

Self-igniting compositions of various kinds have for many years found use in the construction of assorted tools of war for use against personnel and property. More recently it has been recognized that self-igniting compositions are useful as propellants for rockets, guided missiles and aircraft powered by jet or thrust engines. Further, self-igniting compositions are useful in initiating combustion in areas in which the usual methods of initiating combustion can be employed only with great difficulty and inconvenience if at all. For example, self-igniting compositions may be employed to initiate combustion in depleted oil-bearing formations to effect secondary recovery of residual oil in the formation by burning a part of the residual oil and recovering any substantial portion of the remaining residual oil by evaporation, cracking and gas drive of the combustion gases at a producing well.

Hypergolic fuels are useful in the operation of thrust engines. Hypergolic fuels may be generally described as mixtures of a reducing component and an oxidizing component. The individual components of the hypergolic fuel are not self-igniting, but when the two components are mixed there is a short period during which relatively slow reaction of the two components apparently occurs, and this relatively slow reaction is followed by spontaneous ignition of the mixture. Practically all hypergolic mixtures have short ignition delay periods substantially less than 1 second and preferably not more than about 50 milliseconds. The reducing component of a hypergolic fuel should have certain properties, as follows: It should ignite spontaneously upon being combined with the selected oxidizing agent; the ignition delay period should be short, preferably not exceeding 50 milliseconds; it should have a low freezing point so that it can be pumped to the combustion chamber at the low temperatures prevailing at high altitudes; it should have a high boiling point to facilitate handling and increase its safety in use; it should be chemically stable in storage; it should have a relatively low viscosity at low temperatures; it should form gaseous oxidation products and the average molecular weight of these products should be as low as possible in order that the specific impulse (pounds thrust/pounds propellant/second) be high. In addition to the foregoing properties, it is desirable that self-ignition of the mixture of the reducing component and the oxidizing agent be rapid over a wide temperature range; that the reducing component have a high density so that the volume of fuel tanks may be reduced; that the material be non-toxic and easy to handle; that it have a high heat of combustion; and that it be non-corrosive.

It has now been found that a fire can be started by rapid auto-ignition by mixing at least one material of the group consisting of mercaptals and mercaptols containing 3 to 12 carbon atoms per molecule with fuming nitric acid.

In one embodiment of the invention a thrust engine is operated by passing a material of the group consisting of mercaptals and mercaptols containing 3 to 12 carbon atoms per molecule and fuming nitric acid into the com-

## 2

bustion chamber of the engine to form an ignited propulsive charge and ejecting the gases formed by burning charge from the chamber at high velocity.

It has further been found that a mixture consisting of essentially about 75% by weight of isopropylidene diethyl mercaptol and about 25% by weight ethylidene diethyl mercaptol possess an extraordinary combination of physical and chemical properties which make the mixture extremely valuable as the reducing component of a hypergolic fuel.

The mercaptals and mercaptols of the invention are readily prepared by the reaction of a mercaptan with an aldehyde or ketone according to the following equation:

15



where R is an alkyl radical, R' is an organic radical, of the type illustrated in the following Table I, and R'' is either an alkyl radical or hydrogen. A single mercaptan or a mixture of lower mercaptans may be employed in the reaction. Usually a small amount of an acid catalyst is used.

25 A number of mercaptals and mercaptols were prepared by reacting mercaptans with carbonyl compounds, and these materials were tested for self-ignition by a simple drop test. In this test, the mercaptals and mercaptols were dropped from a capillary pipette into a pool of concentrated (95—100%) nitric acid contained in the bottom of a Pyrex tube. As standard quantities, 0.13 cc. of the organic compound and 0.40 cc. of nitric acid are used. Spontaneous ignition is indicated by a flash of light in the bottom of the Pyrex tube. Occasionally when testing a 30 fuel and it is found that ignition does not occur, activity of a fuel may be indicated by the evolution of fumes and heat from the mixture. The drop tests are conducted at room temperature. The results of drop tests of a number of mercaptals and mercaptols in the manner above described are reported in the following Table I. Instead of setting out the chemical names of the mercaptals and mercaptols, their composition is indicated by listing the carbonyl component and the mercaptan component from which they were made according to the above equation.

45

TABLE I  
Drop tests of mercaptals and mercaptols  
with concentrated  $\text{HNO}_3$

|    | Carbonyl Component  | Mercaptan Component                            |                             |
|----|---------------------|------------------------------------------------|-----------------------------|
| 50 | Butyraldehyde       | n-Butyl Mercaptan                              | ignited.                    |
|    | Crotonaldehyde      | do                                             | Do.                         |
|    | Acetone             | do                                             | Do.                         |
|    | Furfural            | do                                             | Do.                         |
|    | Do                  | do                                             | Do.                         |
| 55 | Butyraldehyde       | t-Butyl Mercaptan                              | Do.                         |
|    | Crotonaldehyde      | n-Decyl Mercaptan                              | no ignition, slow reaction. |
|    |                     | Mixed C <sub>2</sub> —C <sub>4</sub> Mercaptan | ignited.                    |
| 60 | Furfural            | do                                             | Do.                         |
|    | Crotonaldehyde      | Allyl Mercaptan                                | Do.                         |
|    | Furfural            | do                                             | Do.                         |
|    | Acetaldehyde        | Methyl Mercaptan                               | Do.                         |
|    | Acetone             | do                                             | Do.                         |
| 65 | Formaldehyde        | do                                             | Do.                         |
|    | Acetaldehyde        | do                                             | Do.                         |
|    | Formaldehyde        | Ethyl Mercaptan                                | Do.                         |
|    | Acetaldehyde        | do                                             | Do.                         |
|    | Do                  | do                                             | Do.                         |
|    | Acetone             | do                                             | Do.                         |
|    | Methyl Ethyl Ketone | do                                             | Do.                         |
| 70 | Acetaldehyde        | Allyl Mercaptan                                | Do.                         |
|    | Benzaldehyde        | Ethyl Mercaptan                                | Do.                         |
|    |                     | Methyl Mercaptan                               | Do.                         |

From the above table it is clear that mercaptals and mercaptols containing 3 to 12 carbon atoms per molecule spontaneously ignite when mixed with concentrated nitric acid.

In order that a hypergolic mixture be useful as a thrust engine fuel, it is not sufficient that the mixture undergo self-ignition. In addition, it is necessary that the ignition delay period, i.e., the time elapsing between the mixing of the two components and the occurrence of spontaneous ignition be extremely short, i.e., less than 50 milliseconds. Further, it is necessary that this short ignition delay period be obtained at low temperatures, for example -40 to -70° F., since temperatures in this range are commonly encountered in high altitude operation of aircraft powered by thrust engines. The following Table II shows ignition delay periods of a number of mercaptals and mercaptols at low temperature. The ignition delay is measured by mixing the mercaptal or mercaptol with the oxidizer in a specially constructed cylinder so arranged that at the instant of mixing the organic compound and the oxidizer an electrode is grounded transmitting a pulse to an electronic timer to commence the measurements of the delay. Soon after the acid contacts the organic material the ignition takes place. Ionization caused by the flame grounds the tubular electrode to the walls of the oxidizer cylinder transmitting a second pulse to the electronic timer to complete the measurement of the delay period.

5

10

15

20

25

30

35

40

45

50

55

60

65

70

75

It will be noted that the blend has a substantially lower viscosity than either of the individual components at -70° F. and that the freeze point of the blend is substantially lower than the freeze point of the mercaptol component.

The ignition delay periods of the individual mercaptol and mercaptal and of blends of the two materials are illustrated in the following Table IV:

TABLE IV

*Ignition delays of various blends of ethyl mercaptal of acetaldehyde and ethyl mercaptol of acetone at -70° F. using red fuming nitric acid as the oxidizer*

| Composition of Fuel Blend (Vol. Percent) |           | Average Ignition Delay (ms.) |
|------------------------------------------|-----------|------------------------------|
| Mercaptal                                | Mercaptol |                              |
| 100                                      | 0         | 47                           |
| 50                                       | 50        | 31.5                         |
| 25                                       | 75        | 26.5                         |
| 0                                        | 100       | 1.26                         |

<sup>1</sup> Supercooled.

TABLE II  
*Ignition delays of low molecular weight mercaptals and mercaptols using low-freezing WFNA or a WFNA-alkane sulfonic acid blend as the oxidizer*

| Fuel, reaction product of— |                     | Oxidizer                                             | Temp., °F. | Ignition delay (ms.) |
|----------------------------|---------------------|------------------------------------------------------|------------|----------------------|
| Mercaptan Component        | Carbonyl component  |                                                      |            |                      |
| Methyl                     | Acetaldehyde        | Low-freezing WFNA <sup>1</sup>                       | -40        | 100                  |
|                            | Acetone             | do                                                   | -40        | 90                   |
|                            | Formaldehyde        | do                                                   | -40        | 5,000                |
|                            | Acetaldehyde        | 80% HNO <sub>3</sub> -20% Ethane Sulfonic Acid       | -40        | 10                   |
|                            | do                  | 80% HNO <sub>3</sub> -20% Methane Sulfonic Acid      | -40        | 9                    |
|                            | do                  | do                                                   | -70        | 21                   |
|                            | Acetone             | 80% HNO <sub>3</sub> -20% Ethane Sulfonic Acid       | -40        | 100                  |
|                            | Formaldehyde        | 85% HNO <sub>3</sub> -15% Methane Sulfonic Acid      | -40        | 18.5                 |
|                            | Acetaldehyde        | do                                                   | -40        | 8                    |
|                            | Acetone             | do                                                   | -40        | 11                   |
| Ethyl                      | Methyl Ethyl Ketone | do                                                   | -70        | 78                   |
|                            | Acetaldehyde        | 85% HNO <sub>3</sub> (99%)-15% Methane Sulfonic Acid | -70        | 46                   |
| Allyl                      | Acetone             | 85% HNO <sub>3</sub> -15% Methane Sulfonic Acid      | -70        | 100                  |
|                            | Acrolein            | 85% HNO <sub>3</sub> -15% Methane Sulfonic Acid      | -70        | 100                  |

<sup>1</sup> Low-freezing WFNA contains 92% HNO<sub>3</sub>, 4% NaNO<sub>2</sub> and 4% H<sub>2</sub>O.

As indicated above, a mixture of the mercaptol formed from ethyl mercaptan and acetone and the mercaptol formed from ethyl mercaptan and acetaldehyde, i.e., a mixture of isopropylidene diethyl mercaptol and ethylidene diethyl mercaptol is an especially efficient reducing component of a hypergolic mixture suitable for use in thrust engines. The properties of the mercaptal, the mercaptol and the blend are set forth in the following Table III:

TABLE III

*Some physical properties of ethyl mercaptol of acetone (isopropylidene diethyl mercaptol), ethyl mercaptal of acetaldehyde (ethylidene diethyl mercaptal), and a 75-25 blend of the mercaptol and mercaptal*

|                        | Ethyl Mercaptol of Acetone | Ethyl Mercaptal of Acetaldehyde | 75-25 Blend of Mercaptol and Mercaptal |
|------------------------|----------------------------|---------------------------------|----------------------------------------|
| Specific Gravity at:   |                            |                                 |                                        |
| 70° F.                 | 0.9468                     | 0.9669                          | 0.9499                                 |
| 0° F.                  |                            |                                 | 0.9853                                 |
| -40° F.                |                            |                                 | 1.0064                                 |
| -70° F.                |                            |                                 | 1.0210                                 |
| Viscosity (Cstks.) at: |                            |                                 |                                        |
| 70° F.                 | 2.45                       | 2.70                            | 1.206                                  |
| 0° F.                  |                            |                                 | 2.495                                  |
| -40° F.                | 4.65                       | 5.76                            | 5.124                                  |
| -70° F.                | 11.98                      | 13.24                           | 10.05                                  |
| Freezing Point, °F.    | -49                        | -117                            | -73                                    |

From the data in Table IV it will be seen that the ignition delay period of a 75-25% blend of the mercaptol and mercaptal has an average ignition delay period of 26.5 milliseconds, i.e., substantially lower than that of the mercaptal component and the blend is a stable liquid at -70° F.

The mercaptals and mercaptols of the invention form hypergolic mixtures with concentrated nitric acid. Commercial nitric acid having a purity in the range from 95 to 100% HNO<sub>3</sub> by weight is a satisfactory oxidizing agent. White fuming nitric acid composed of 98.5% by weight HNO<sub>3</sub> and 1.5% by weight of water is an effective oxidizing agent. Minor proportions of ignition accelerators or freeze point depressants may be added to the nitric acid which is mixed with the mercaptals and mercaptols to cause spontaneous ignition of the mixture. For example, 2 to 20% by weight of nitrogen dioxide may be dissolved in the nitric acid. This mixture is sometimes referred to as red fuming nitric acid. 2 to 20% by weight sulfuric acid may be added to the nitric acid to accelerate ignition. 2 to 20% of nitrosyl sulfuric acid may be added to the nitric acid as an ignition accelerator. 5 to 25% by weight of a lower alkane sulfonic acid such as methane sulfonic acid, ethane sulfonic acid, and the like, may be added to the nitric acid to produce a mixture characterized by a much reduced freeze point and good ignition properties when mixed with the mercaptals and mercaptols. Nitric acid containing a small amount up to about 4% by weight of sodium nitrite and a small amount up to about

4% by weight of water has a low freeze point and forms hypergolic mixtures with the mercaptals and mercaptols of the invention.

If the mixtures of nitric acid and mercaptals and mercaptols are to be employed as a thrust engine fuel, it is desirable that the mixture contain approximately the quantity of nitric acid stoichiometrically required for complete oxidation of the organic material to water, carbon dioxide and sulfur dioxide. Maximum thrust appears to be obtained if the nitric acid is present in the mixture at about 85 to 95% of the amount stoichiometrically required for complete oxidation. Where it is simply desired to employ a mixture of mercaptal or mercaptol with nitric acid to start a fire, as, for example, when such a mixture is introduced into the bottom of an oil well to initiate burning in the formation, the proportions of the two components may be varied rather widely, for example, mixtures containing the organic compound and the nitric acid at weight ratios from 1:5 to 5:1 may be employed.

We claim:

1. The method of starting a fire by auto-ignition, which comprises mixing a material having the formula:



wherein R and R' are materials selected from the group consisting of alkyl radicals and alkenyl radicals and R'' is a material selected from the group consisting of alkyl radicals, alkenyl radicals and hydrogen and wherein the total number of carbon atoms is in the range 3 to 12 with sufficient concentrated nitric acid to form a mixture containing said material and nitric acid at a weight ratio within the range 1:5 to 5:1.

2. A fuel characterized in that it ignites spontaneously when mixed with fuming nitric acid consisting essentially of about 75% by weight of isopropylidene diethyl mercaptol and about 25% by weight of ethylidene diethyl mercaptol.

References Cited in the file of this patent

15 Hackh's Chemical Dictionary, 3rd edition (1944), The Blakiston Co., Philadelphia, pages 598, 599.

The Van Nostrand Chemist's Dictionary, D. Van Nostrand Co., Inc., N.Y. (1953), pages 458, 459.